# EUROPEAN PATENT SPECIFICATION

(11) **EP 0 144 438 B1**
(45) Date of publication and mention of the grant of the patent: **10.08.1988**
(21) Application number: 84902055.7
(22) Date of filing: 18.05.1984
(51) Int. Cl.: B41M 5/12

(54) **PROCESS FOR PRODUCING PRESSURE-SENSITIVE SHEET MATERIAL**
VERFAHREN ZUR HERSTELLUNG VON DRUCKEMPFINDLICHEM BLATTMATERIAL
PROCEDE DE PRODUCTION D'UN MATERIAU EN FEUILLE SENSIBLE A LA PRESSION

(30) Priority: 21.05.1983 JP 89644/83
(43) Date of publication of application: 19.06.1985
(73) Proprietor: MITSUBISHI PAPER MILLS, LTD., Chiyoda-ku Tokyo 100 (JP)
(72) Inventor: SENOH, Hideaki Mitsubishi Seishi Takasago-Ryo, Hyogo 676 (JP); KOSAKA, Takao 2108, Mikage, Hyogo 679-21 (JP); KAGOTA, Nobuhiro Mitsubishi Seishi Sakaemachi, Takasago-shi Hyogo 676 (JP)
(74) Representative: Hansen, Bernd, Dr. Dipl.-Chem.
(86) International application number: JP8400248
(87) International publication number: WO8404728

(56) References cited:
- FR-A- 2 404 533
- JP-A-51 034 013

## Description

### Technical Field

This invention relates to a novel method of making pressure sensitive sheet materials. More particularly, it relates to an improvement in the method for making pressure sensitive sheet materials, such as carbonless pressure sensitive recording paper and pressure sensitive adhesive sheet, comprising a support in sheet form and, provided thereon, a coating of pressure-rupturable microcapsules.

### Background Art

There are known a large variety of pressure sensitive sheet materials. A typical example is a carbonless pressure sensitive recording paper utilizing the color reaction which takes place in a solvent medium between a colorless dye and a color developer such as activated clay, acid clay, phenol resins, aromatic carboxylic acids or metallic salts thereof.

Examples of carbonless pressure sensitive recording sheets include a combination type comprising, on one hand, a sheet carrying a coating formed by emulsifying a solution of a colorless dye dissolved in a solvent, encasing the emulsified finely divided liquid particles in protective pellicles of natural or synthetic polymers (i.e. microencapsulation), and coating the resulting microcapsule suspension on a support, and, on the other hand, a sheet comprising a support and, provided thereon, a coating of color developers; and a single-layer type comprising a support and, provided thereon, a coating containing both the said microencapsulated colorless dye and the color developer or microencapsulated color developer. There is also known another combination-type carbonless pressure sensitive recording paper comprising a sheet carrying a coating of microencapsulated solution of a color developer and a sheet carrying a coating of a colorless dye.

Other pressure sensitive sheet materials than the carbonless recording paper include a pressure sensitive adhesive sheet carrying a coating of adhesive-containing microcapsules or a coating of solvent- containing microcapsules and an adhesive, and an encapsulated perfume sheet carrying a coating of microencapsulated perfume.

The carbonless pressure sensitive recording sheet materials, which are commercially manufactured on the largest scale of all other pressure sensitive sheet materials, are now in use in various commodity areas such as computer output recording sheets, business slips, and business manifolding forms, and are required to have performance characteristics which comply with the requirements of particular uses. For this reason, in preparing the microcapsule dispersion, various auxiliary agents are added to meet various requirements. Above all, many proposals have heretofore been made to use, as stilt material, powdered pulp, starch powder, glass beads, plastic beads, talc, calcium carbonate, and clays for the purpose of enhancing the resistance of the microcapsule-coated sheet materials against those unintentional pressing, scuffing, impact, and the like which would cause smudging due to rupture of the microcapsules during manufacture, handling, printing, or actual use of the microcapsule-coated sheet.

Examples of proposed stilt materials for use in carbonless pressure sensitive recording paper include fine powders of starch derivatives (Japanese Patent Publication No. 1,178/72), starch grains having an average diameter as large as at least about 1.2 times the microcapsule diameter (Japanese Patent Publication No. 33,204/73), corncob (waste part of an ear of corn after removal of corn grains) [Japanese Patent Application No. 16,708/73], microspheres expandable by heating [Japanese Patent Application No. 32,013/73], starch grains of large diameter derived from beans other than soybean [Japanese Patent Application No. 34,013/76], acid-modified polyolefin particles [Japanese Patent Application No. 111,810/ 78], water-insoluble vegetable proteins [Japanese Patent Application No. 58,510/79], and FR-A-2 404 533 (soybean powder), finely powdered polyolefin [Japanese Patent Application No. 51,611/79], finely powdered polyolefin for use in self-contained pressure sensitive recording paper of the single layer type [Japanese Patent Application No. 3,969/80], powdered cellulose (US Patent 2,711,375), and finely powdered starch (Brit. P. 1,232,347).

Stilt materials generally used forthe purpose of preventing the recording sheet from the smudging due to unintentional rupture of the microcapsules are finely powdered cellulose, finely powdered raw starch, talc, kaolin, bentonite, pyrophyllite, and inorganic pigments such as zinc oxide, titanium oxide, and alumina.

As described above, for the purpose of preventing the carbonless pressure sensitive recording paper from smudging due to unintentional rupture of microcapsules during manufacture, fabrication, printing, or actual use of the recording paper, various proposals have been made and helpful in bringing about a certain degree of improvement. In particular, powdered pulp (finely powdered cellulose) and starch grains are excellent, practical stilt materials and are now in worldwide use. However, the use of powdered pulp as stilt material involves various problems such as a difficulty encountered in coating operation resulting from the increase in viscosity of the coating composition during the coating operation, rendering the uniform distribution of stilt material difficult, resulting in, on one hand, stilt-rich coating areas, where the smudging becomes reduced, while the color developing performance becomes deteriorated and, on the other hand, stilt-poor coating areas where the smudging becomes so enhanced that sufficient performance characteristics are no more obtained from the practical view point.

Therefore, an object of this invention is to provide a method of making pressure sensitive sheet materials which are lessened in susceptibility to the unintentional rupture of microcapsules and the attendant smudging, to an extent sufficient for practical use, while the color developing function being retained or improved.

Another object of this invention is to provide a method of making pressure sensitive sheet materials, according to which it is possible to retard the viscosity increase in the coating composition during manufacture or application and to minimize the fluctuation in component distribution of the coating composition in order to keep the coating surface from deterioration in quality or to keep the distribution of stilt materials uniform throughout the coating composition.

The invention comprises a method for production of a pressure sensitive sheet material by coating pressure-rupturable microcapsules and a soybean powder on a sheet support, and is characterized in that said defatted soybean powder on a sheet support, and is characterized in that said defatted soybean powder has a protein content of from 45 to 55% per weight and a water-soluble nitrogen content of from 5 to 15% per weight ofthetotal nitrogen content and has been produced by treating and modifying a solvent-extracted soybean powder with an alcohol.

When the defatted soybean powder obtained by treating and modifying defatted soybean with an alcohol is used as the stilt material, the coating composition is kept from viscosity increase during its manufacture and retains desirable fluidity so as to improve spreadability of the composition; moreover, owing to sufficient water-retentivity. of the alcohol-treated defatted soybean powder, the fluctuation in component distribution is kept low throughout the coating composition so that after application of the composition, there is obtained a coat of uniform surface quality. For instance, in the case of a carbonless pressure sensitive recording paper of color developing quality at normal level, the alcohol-treated defatted quality at normal level, the alcohol-treated defatted soybean powder exhibits distinguished stilt effect so that the unintentional rupture of microcapsules and the attendant smudging under light pressing can be minimized.

### Description of the Preferred Embodiment

The invention is described in detail in the following.

The defatted soybean in powder form contains proteins, fats, fibrous matters, ash; polysaccharides such as galactan and pentosan; saccharides such as sucrose, stachyose, and raffinose; and vitamins.

In manufacturing the defatted soybean, it is general practice to remove, in the first step, fatty matters fromthe raw soybean by expression or solvent extraction. Since the removal of fatty matters by expression is insufficient, it has recently become a common practice to use the solvent extraction which reduces the residual fatty matter content of the defatted soybean down to 1 % or below. In the extraction, benzene and n-hexane are generally used as the defatting solvent. The treated soybean is stripped of the solvent by treating with steam at elevated temperatures or by treating under reduced pressure or with a solvent vapor at low temperatures.

The defatted soybean powder used in this invention is obtained from the solvent-extracted soybean by treating with alcohols such as methanol, ethanol, and propyl alcohol. If the defatted soybean produced by expression is used as stilt material, owing to the residual oil which amounts to about 8%, there will occur in the coating layer a phenomenon of cissing which hinders uniform distribution of the stilt material. The defatted soybean powder used in this invention is that obtained from the solvent-extracted soybean by treating and modifying with an alcohol to adjust the protein content to 45 to 55%, the water-soluble nitrogen content being 5 to 15% of the total nitrogen content. Such a defatted soybean powder is an effective stilt material and, in addition, has an advantage of improving the water retentivity of the capsule- containing coating composition on account of the presence of water-soluble constituents. If the water-soluble nitrogen content exceeds 15% of the total nitrogen, gelation will take place in the coating composition, whereas if the content is below 5%, the water retention becomes insufficient. The principal object of treating and modifying the defatted soybean with an alcohol is deodorizing and decoloring. The resulting defatted soybean powder is a powder material which is nonsticky, easy to handle, and pale amber yellow in color. As a consequence, the coating layer containing such a stilt material is excellent in surface brightness.

A powder material prepared by dissolving raw soybean or defatted soybean in an alkali solution and reprecipitating with an acid, as known from FR-A-2 404 533, which is the nearest prior art document, is generally a high-purity (e.g. 85%) protein substance and substantially devoid of water-solubility, the water-soluble nitrogen content being 1% of the total nitrogen or less. For this reason, as ascertained by the present inventors, such as soybean powder is unsuitable for actual use, because if it is added to a capsule- containing coating composition, the composition becomes less uniform in component distribution, as compared with the composition prepared according to this invention.

The defatted soybean powder used in this invention is amorphous in particle shape and has an average particle size of from 10 to 60 um, especially preferred size being 20 to 30 !-1m which are larger than the capsule size, though not limitative. If necessary, the defatted soybean powder can be used in combination with other known stilt materials such as, for example, finely powdered cellulose or wheat starch to obtain also a desirable result.

Typical examples of the processes for producing microcapsules used in this invention are physical, coacervation, interfacial polymerization, and in situ polymerization processes.

In the case of carbonless pressure sensitive recording paper, typical examples of colorless dyes enclosed in the capsules include phthalides such as 3,3-bis(4-dimethylaminophenyl)-6-dimethylaminophthalide and 3,3-bis(1,2-dimethylindol-3-yl)-5-dimethylaminophthalide; fluoranes such as 3-diethylamino-6-methyl-7-anilinofluorane, 3-(N-methyicyciohexytamino)-6-methyi-7-aniiinofiuorane, 3-diethylamino-6-methyl-7-chlorofluorane, 3-diethylamino-6-methyl-7-chlorofluorane, and 3-diethylamino-7-dibenzylaminofluorane; thiazine compounds such as benzoylleuco methylene blue; lactams such as N-(p-nitrophenyl)-rhodamine B lactam; spiro compounds such as 1,3,3-trimethylindolinospiropyrane; and indolyl red. As for the pellicle materials for microcapsules, there may be mentioned, nonlimitatively, unmodified or partially modified natural polymers such as gelatin, cellulose derivatives, and starch derivatives; and synthetic resins such as urea-formaldehyde resin, melamine-formaldehyde resin, reaction products of isocyanate compounds and hexamethylenediamine, and reaction products of adipic acid dichloride and hexamethylenediamine. However, in view of the reinforcement of capsule wall properties such as heat resistance, solvent resistance, water resistance, chemical resistance, and impact resjstance, microcapsules covered with synthetic resins are preferred.

As oily substances which constitute the internal phase of microcapsules, there may be used solvents of high boiling points which can be at least one selected from natural oils such as petroleum- or mineral-base oils, and animal- or vegetable-base oils or from synthetic oils. Especially preferred are those which dissolve the colorless dyes. As examples, mention may be made of alkylated biphenyls, alkylated terphenyls, alkylated naphthalenes, triarylmethanes, diarylalkanes, phthalic esters, phosphoric esters, sulfonic esters, diaryl ethers, and higher alkylbenzenes, but the invention is not limited thereto.

The pressure sensitive sheet material manufactured according to this invention comprises at least a support, microcapsules, and a defatted soybean powder obtained from the solvent-extracted soybean by treating and modifying with an alcohol. In addition to the microcapsules and the said defatted soybean powder, the present sheet material may contain binders including water-soluble natural binders such as starch and carboxymethylcellulose; and water-soluble synthetic binders such as polyvinyl alcohol, polyvinylpyrrolidone, and polyacrylic acid; and latices such as styrene-butadiene latex, styrene-butadiene- acrylic acid latex, butadiene rubber latex, and neoprene rubber latex. Further, if necessary, there may be added, as lubricant or extender, inorganic pigments such as talc, titanium dioxide, zinc oxide, calcium carbonate, and activated clay; and organic lubricants such as ethylene-bisstearamide.

The coating composition of this invention can be applied by any of the known techniques such as, for example, air knife coating, blade coating, bill blade coating, roll bar coating, three-applicator-roll coating, and curtain coating. In general, the blade coating is effectively used in applying a high-solid content coating composition. The coating composition of this invention can be efficiently applied also by the blade coating technique, because even at high solids concentration, it is hardly subject to fluctuation in distribution of components and has excellent fluidity.

The defatted soybean powder and the microcapsules should be present on the same side of the support. Therefore, it can be added to the coating composition which is to form the microcapsule layer, or to the coating composition which is to form an under- and/or over-layer to the microcapsule layer.

As examples of commercial solvent extracted soybean powder products, mention may be made of "S-Sanmeat" (Ajinomoto Co.) extra grade (7.0% of water, 54.0% of protein, and 0.2% of oil) and first grade (7.5% of water, 49.0% of protein, and 0.2% of oil).

The invention is illustrated below in detail with reference to Example, but the invention is not limited thereto. Hereinafter all parts are by weight.

### Example

### (Alcohol-treated defatted soybean powder was used.)

### Example of microcapsule preparation:

The above solution of an electron donating leuco dye in the high-boiling solvent was emulsified in 100 parts of a 5-% aqueous solution of a styrene-maleic acid copolymer. An aqueous solution of melamine-formaldehyde prepolymer was prepared by heating a mixture (adjusted to pH 9.5 with sodium hydroxide) of 10 parts of melamine, 25 parts of 37-% formalin, and 20 parts of water. The prepolymer solution was added to the above emulsion and allowed to react with stirring at 75°C for 90 minutes. The reaction mixture was cooled to room temperature and adjusted to pH 9.5 with sodium hydroxide to obtain a microcapsule dispersion. To 100 parts (dry basis) of the dispersion, was added 35 parts of a defatted soybean powder ("S-Sanmeat" extra grade, a product of Ajinomoto Co.; a soybean powder produced by treating solvent-defatted soybean with an alcohol), 35 parts of talc,17 parts of polyvinyl alcohol, and 17 parts (dry basis) of a styrene-butadiene latex. The mixture was thoroughly stirred to form a dispersion. The dispersion was coated by means of an air knife coater on a plain paper (40 g/m² in basis weight) at a coverage of 5 g/m² (dry basis) to obtain an upper sheet for a carbonless pressure sensitive recording paper.

### Comparative Example 1

### (Wheat starch was used.)

An upper sheet was obtained in the same manner as in Example, except that 35 parts of wheat starch was used in place of the defatted soybean powder treated with an alcohol.

### Comparative Example 2

### (Finely powdered cellulose was used.)

An upper sheet was obtained in the same manner as in Example, except that 35 parts of finely powdered cellulose was used in place of the defatted soybean powder treated with an alcohol.

### Comparative Example 3

### (No stilt material was used.)

An upper sheet was obtained in the same manner as in Example, except that the defatted soybean powder treated with an alcohol was omitted and each 13 parts of polyvinyl alcohol and a styrene-butadiene latex were used as binder for 100 parts of the capsules, the coverage with respect to capsules being the same as in Example.

### Comparative Example 4

### (Defatted soybean not treated with an alcohol was used.)

An upper sheet was obtained in the same manner as in Example, except that 35 parts of solvent-defatted soybean (50% in protein content) not treated with an alcohol was used in place of the defatted soybean powder treated with an alcohol.

### Comparative Example 5

### (Water-insoluble soybean protein powder was used.)

An upper sheet was obtained in the same manner as in Example, except that 35 parts of a high-purity soybean protein powder having a water-insoluble protein content of about 85% or above was used in place of the defatted soybean powder treated with an alcohol.

### Color developer sheet:

A pressure sensitive recording sheet (Mitsubishi NCR paper CF) carrying a coating of an electron accepting solid acid (oil-soluble novolak-type phenol resin) was used as color developer sheet (under sheet). The upper sheet was placed on the under sheet so as to bring both coated sides in contact with each other and tested for coloring characteristics and smudge characteristics. The test results were as shown in the table. The test results for smudge characteristics were as shown in the table.

In the table, the coloring intensity is the intensity of color measured after one hour of pressure application at 90 kg/cm by means of a calender. The smudge is expressed in terms of reflectance measured 24 hours after rubbing under a load of 450 g/cm^{3.} All numerical values were corrected for the background condition. Marks, o and X, were the results of visual inspection performed at the same time.

As is apparent from the table, a recording paper system comprising a powder material obtained by treating and modifying the solvent-defatted soybean with an alcohol showed especially well-balanced practical characteristics, being excellent in coloring characteristics, less subject to smudging, low in viscosity of the coating composition, and less subject to the fluctuation of component distribution in the coating composition.

### Possibility of Industrial Application

As described in the foregoing, the method of this invention is suitable for the production of carbonless pressure sensitive recording paper, pressure sensitive adhesive sheet, perfume-containing capsule sheet, and the like. Above all, it is especially suited for the production of pressure sensitive recording paper, because it keeps the recording paper from smudging due to uninternational rupture of the microcapsules.

## Claims

1. A method for the production of a pressure sensitive sheet material by coating pressure-rupturable microcapsules and a soybean powder on a sheet support, characterized in that said defatted soybean powder has a protein content of from 45 to 55% per weight and a water-soluble nitrogen content of from 5 to 15% per weight of the total nitrogen content and has been produced by treating and modifying a solvent-extracted soybean powder with an alcohol.

2. A method for the production of a pressure sensitive sheet material according to Claim 1, characterized in that the defatted soybean powder has an average particle size of 10 to 60 pm.

3. A method for the production of a pressure sensitive sheet material according to Claim 1, characterized in that the coating composition which provides the coating layer containing a defatted soybean powder has been obtained by adding said defatted soybean powder to a microcapsule-containing coating composition.

4. A method for the production of a pressure sensitive sheet material according to Claim 1, characterized in that the coating composition which provides the coating layer containing the defatted soybean powder contains no capsule and is coated over and/or under the microcapsule layer.

## Patentansprüche

1. Verfahren zur Herstellung eines druckempfindlichen Blattmaterials, bei dem man durch Druck zerbrechbare Mikrokapseln und Sojapulver auf einen Blattträger beschichtet, dadurch gekennzeichnet, dass das entfettete Sojabohnenpulver einen Proteingehalt von 45 bis 55 Gew.% und einen Gehalt an wasserlöslichem Stickstoff von 5 bis 15 Gew.%, bezogen auf dem Gesamtstickstoffgehalt, aufweist und hergestellt wurde, indem man ein lösungsmittelextrahiertes Sojabohnenpulver mit einem Alkohol behandelte und modifizierte.

2. Verfahren zur Herstellung eines druckempfindlichen Blattmaterials gemäss Anspruch 1, dadurch gekennzeichnet, dass das entfettete Sojabohnenpulver eine durchschnittliche Teilchengrösse von 10 bis 60 11m hat.

3. Verfahren zur Herstellung eines druckempfindlichen Blattmaterials gemäss Anspruch 1, dadurch gekennzeichnet, dass die Überzugszusammensetzung, mit welcher die Überzugsschicht, welche das entfettete Sojabohnenpulver enthält, hergestellt wird, erhalten wurde, indem man das entfettete Sojabohnenpulver zu einer Mikrokapseln enthaltenden Überzugszusammensetzung gibt.

4. Verfahren zur Herstellung eines druckempfindlichen Blattmaterials gemäss Anspruch 1, dadurch gekennzeichnet, dass die Überzugszusammensetzung, welche die das entfettete Sojabohnenpulver enthaltende Überzugsschicht ergibt, keine Kapseln enthält und über und/oder unter die Mikrokapselschicht aufgebracht wird.

## Revendications

1. Procédé de production d'un matériau en feuille sensible à la pression, par enduction, sur une feuille support, d'une poudre de soja et de microcapsules frangibles sous l'effet d'une pression, caractérisé en ce que ladite poudre de soja dégraissée présente une teneur en protéines de 45 à 55% en poids et une teneur en azote hydrosoluble de 5 à 15% en poids par rapport à la teneur totale en azote, et en ce qu'elle a été produite par traitement et modification, par un alcool, d'une poudre de soja ayant subi une extraction par solvant.

2. Procédé de production d'un matériau en feuille sensible à la pression, conforme à la revendication 1, caractérisé en ce que la poudre de soja dégraissée présente une dimension moyenne de particules de 10 à 60 pm.

3. Procédé de production d'un matériau en feuille sensible à la pression, conforme à la revendication 1, caractérisé en ce que la composition d'enduction, qui fournit la couche d'enduction contenant la poudre de soja dégraissée, a été obtenue par addition de ladite poudre de soja dégraissée à une composition d'enduction contenant des microcapsules.

4. Procédé de production d'un matériau en feuille sensible à la pression, conforme à la revendication 1, caractérisé en ce que la composition d'enduction, qui fournit la couche d'enduction contenant la poudre de soja dégraissée, ne contient pas de capsules et est étalée par-dessus et/ou par-dessous la couche de microcapsules.
